# EUROPEAN PATENT APPLICATION

(11) **EP 3 499 161 A1**
(43) Date of publication of application: **19.06.2019**
(21) Application number: 17206951.0
(22) Date of filing: 13.12.2017
(51) Int. Cl.: F27B 3/28, F27D 19/00, F27D 21/00

(54) **METHOD OF CONTROLLING A GAS FURNACE FOR MELTING METAL AND CONTROL SYSTEM THEREFOR**

(71) Applicant: Novamet Sàrl, 1004 Lausanne (CH)
(72) Inventor: ROSTAMIAN, Amin, 1004 Lausanne (CH); RAPPAZ, Michel, 1006 Lausanne (CH)
(74) Representative: reuteler & cie SA

(57) **Abstract**

A method of controlling a metal melting process in a gas furnace (3) with a control system (2), the gas furnace comprising a furnace chamber (9) enclosed by walls (5a, 5b, 5c) and a door (7), gas burners (11) configured to heat the metal (1) loaded in the chamber, a flue gas exit (13) and a plurality of sensors (15) including at least one temperature sensor at a top wall (5a) of the furnace chamber and at least one temperature sensor (15d) to measure the metal temperature in its melted state. The method comprises:
a) receiving in the control system during the melting process, process parameter measurements from said sensors including at least one temperature sensor,
b) simulating in the control system a numerical physical heat exchange model in the furnace including radiation between walls and the metal, conduction though the metal and walls, and convection in the furnace chamber including calculating a temperature at a position in the furnace corresponding to said at least one temperature sensor,
c) comparing the data obtained from the simulated physical heat exchange model with data obtained from the sensor measurements,
d) tuning at least one adjustable parameter of the physical heat exchange model to reduce the difference between compared data,
e) based on the tuned simulated physical heat exchange model, calculating in the control system the change over time of the process parameters, including at least one process parameter which is not directly measured up to the end of the cycle,
f) transmitting to an operator interface (14) of the control system, information on the change over time of predicted process parameters and at least one recommendation for executing a future operation in relation to the furnace at a recommended time.

## Description

### Field of the Invention

This invention relates to a method of controlling a gas furnace for melting metal and a control system therefor. The metal may in particular be aluminium.

### Background of the Invention

The current world production of aluminium is around 120 million tpa (tonne per annum), with about 70 million tonnes produced by secondary production (remelting of aluminium). The secondary production includes melting of aluminium ingot and scrapes in furnaces followed by casting. The melting process carried out in melting furnaces is a costly process which consumes significant amounts of energy and generates significant amounts of CO₂ emissions (approx. 160 kg/tonne).

In a gas furnace, combustion with oxygen in the air of a fossil gas injected in gas burners located in the furnace supplies the enthalpy to the top surface of aluminium (e.g. scrap), previously loaded into the furnace. Thereby, the metal (a load) is heated and melts by both convective and radiative heat transfer mechanisms from the flame to the melt, but also indirectly by radiation from the heated ceramic of the furnace walls and vault. During a melting cycle, the temperature inside the furnace is regulated by adjusting the power output of the burners in such a way as to maintain a nearly constant temperature of the ceramic vault or the flue gas. A thermocouple can be introduced into the melt only once the solid load has been melted, in which case the melt temperature can be used to control the power of the burner.

During a melting cycle, the liquid metal and the solid scrapes can be oxidized to form a dross layer over the melt. The formation of a dross layer reduces the heat transfer from the burners to the metal, and consequently reduces the melting efficiency, but also generates heat by the oxidation reaction.

The efficiency and cost of the melting process thus highly depends on the behavior of the furnace operators. To optimize the melting process which includes several steps, the steps should be performed with an optimal time sequence. Nowadays, the operators determine these time sequences based on their experience and feeling. That introduces huge variations in the process and increases the costs of the operations, as well as energy consumption and CO₂ emissions.

### Summary of the Invention

In view of the foregoing, it is an object of this invention to provide a method and a control system for a gas furnace for melting metal that optimizes the melting process, in particular to reduce energy consumption and process time.

It would be advantageous to provide a method and a control system for a gas furnace for melting metal that provides information on optimal time sequences of process steps on a real-time basis to an operator.

It would be advantageous to provide a method and a control system for a gas furnace for melting metal that enables early detection of abnormalities and faults.

It would be advantageous to provide a method and a control system for a gas furnace for melting metal that provides recommendations for rapid corrective actions during production to operators.

It would be advantageous to provide a method and a control system for a gas furnace for melting metal that provides performance information such as performance statistics.

It would be advantageous to provide a method and a control system for a gas furnace for melting metal that enables retrofit implementation in existing gas furnaces.

Objects of this invention have been achieved by providing the gas furnace control system for melting metal according to claim 12, and a method according to claim 1.

Disclosed herein is a method of controlling a metal melting process in a gas furnace with a control system, the gas furnace comprising a furnace chamber enclosed by walls and a door, gas burners configured to heat the metal loaded in the chamber, a flue gas exit and a plurality of sensors including at least one temperature sensor at a top wall (vault) of the furnace chamber and at least one temperature sensor to measure the metal temperature in its melted state, the method comprising:
a) receiving in the control system during the melting process, process parameter measurements from said sensors including at least one temperature sensor,
b) simulating in the control system a numerical physical heat exchange model in the furnace including radiation between walls and the metal, conduction though the metal and walls, and convection in the furnace chamber including calculating a temperature at a position in the furnace corresponding to said at least one temperature sensor,
c) comparing the data obtained from the simulated physical heat exchange model with data obtained from the sensor measurements,
d) tuning at least one adjustable parameter of the physical heat exchange model to reduce the difference between compared data,
e) based on the tuned simulated physical heat exchange model, calculating in the control system the change over time of the process parameters, including at least one process parameter which is not directly measured up to the end of the cycle,
f) transmitting to an operator interface of the control system, information on the change over time of predicted process parameters and at least one recommendation for executing a future operation in relation to the furnace at a recommended time.

In an advantageous embodiment, the process parameters measured and received by the control system and included in the numerical model further include a flue gas exit temperature.

In an advantageous embodiment, the process parameters measured and received by the control system and included in the numerical model further include a burner gas flow rate.

In an advantageous embodiment, the process parameters measured and received by the control system and included in the numerical model further include a burner gas inlet temperature.

In an advantageous embodiment, the process parameters measured and received by the control system and included in the numerical model further include an air inlet temperature.

In an advantageous embodiment, process parameters measured and received by the control system and included in the numerical model further include any one or more of:
- a chemical composition of at least one component (such as CO₂) of the flue gas,
- a gas pressure inside the furnace chamber,
- a furnace bottom wall temperature.

In an advantageous embodiment, the simulated physical heat exchange model includes calculating in the control system the heat exchange when the door is opened and including the opening of the door in the evolution of the process parameters.

In an advantageous embodiment, the recommended future operation includes any one or more of the operations of:
- loading solid metal in the furnace,
- skimming dross on the surface of the molten metal,
- stirring the molten metal in the furnace,
- introducing a thermocouple in molten metal,
- changing the heat output of the gas burners,
- introducing chemicals in the furnace,
- introducing alloys in the furnace,
- stopping the melting process.

In an advantageous embodiment, the information on the change over time of predicted process parameters transmitting to the operator interface includes a plurality of recommendations for executing said future operations at recommended times up to an end of the melting process.

In an advantageous embodiment, the step of generating the recommended future operation and recommend timing thereof includes accessing a database storing past melting process parameters and executing a learning algorithm on said past melting process parameters.

In an advantageous embodiment, operator feedback on operations on the furnace are input into the operator interface and transmitted from the operator interface to a server of the control system.

In an advantageous embodiment, operator feedback includes information on whether or not operational procedures were executed at the recommended times or postponed.

Also disclosed herein is a control system for a gas furnace for melting metal, adapted to carry out the process according to any one of the previous claims, comprising a melt optimization computing system including:
- a melt optimization control program stored in a memory of the computing system and executable by a processor of the computing system, the melt optimization control program comprising an acquisition module configured to receive process parameters from the sensors, including at least one vault temperature measurement and at least one molten metal temperature measurement, and a simulation module configured to calculate a physical heat exchange model in the furnace including radiation between walls and the metal, conduction though the metal and walls, and convection in the furnace chamber including calculating a temperature at a position in the furnace corresponding to said at least one temperature sensor, the melt optimization program configured to compare acquired process parameters with process parameters calculated by the numerical physical heat exchange model and to tune the model by adjusting at least one parameter thereof in order to reduce the difference between measured and calculated process parameter values; and
- an operator interface comprising a display, configured to receive and display information outputted by the melt optimization program, including information on the change over time of predicted process parameters and at least one recommendation for executing a future operation in relation to the furnace at a recommended time.

In an advantageous embodiment, the operator interface is arranged to display a furnace status panel providing information on the status of process parameters and a recommendation panel providing information on the recommended future operations and the timing thereof.

In an advantageous embodiment, the operator interface is arranged to display a control and further actions panel providing information on the next recommended operation and the timing thereof.

In an advantageous embodiment, the control system further comprises a database in which process parameters of past melting processes are stored, and a learning module receiving data from the database.

Further objects and advantageous aspects of the invention will be apparent from the claims, and from the following detailed description and accompanying figures.

### Brief Description of the drawings

The invention will now be described with reference to the accompanying drawings, which by way of example illustrate the present invention and in which:
Figure 1a is a schematic simplified cross-sectional diagram of a typical gas furnace for melting metal, for instance for melting aluminium scrapes and ingots;
Figure 1b is a schematic simplified diagram of a gas furnace for melting metal used to describe an example of a numerical model used in a heat exchange model according to an embodiment of the invention;
Figure 1c illustrates viewing factors calculation between two surfaces used in a heat exchange model according to an embodiment of the invention;
Figures 2a and 2b are schematic simplified overview diagrams of implementation of a control system for a gas furnace for melting metal according to an embodiment of the invention;
Figure 3 is a schematic simplified diagram of a gas furnace for melting metal connected to a control system for the gas furnace according to an embodiment of the invention;
Figure 4 illustrates schematically examples of data collected by a control system for a gas furnace for melting metal according to an embodiment of the invention;
Figure 5 illustrates schematically a graph of measurements during a melting process collected by a control system for a gas furnace for melting metal according to an embodiment of the invention;
Figure 6 illustrates a graphical operator interface of a control system for a gas furnace for melting metal according to an embodiment of the invention;
Figure 7 is a flowchart illustrating steps of a metal melting process with a gas furnace according to an embodiment of the invention.

### Detailed description of embodiments of the invention

Referring to the figures, a gas furnace system for melting metal 1, for instance for melting aluminium, comprises a gas furnace 3 and a control system 2. The gas furnace 3 comprises a furnace chamber 9 enclosed by walls 5 and a door 7, gas burners 11 configured to heat the metal 1 in the chamber, a flue gas exit 13 and a plurality of sensors 15. The furnace may further comprise a stirrer within the chamber configured to stir the metal in its melted state, in particular an electromagnetically driven stirrer. The door 7 is typically a sliding door through which the metal is loaded. The vault and lateral walls of the furnace are lined with heat resistant ceramic material and the gas burners may typically be mounted on the sidewalls of the chamber above the level of the liquid metal at full capacity. The gas fumes (combustion product) are recovered through the flue gas exit 13 which may be connected to a heat exchanger in order to recover heat energy.

The various heat and mass transfers occurring within a furnace are illustrated schematically in figure 1, such heat transfers including radiation among the walls and metal 1, convection within the chamber, conduction through the metal and the walls, convection and radiation between the flame and walls and metal, and when the door is opened, heat loss by radiation and convection through the opening.

The sensors 15 may include :
a- Sensor 15a indicating that the furnace door is fully open
b- Sensor 15b indicating that the furnace door is fully closed
c- Sensor to measure the inner furnace pressure
d- Thermocouple 15d to measure the metal temperature
e- Thermocouple 15e to measure the temperature on a top side of the chamber (for instance between 3 to 7 thermocouples depending on the furnace)
f- Thermocouple 15f to measure the temperature on the bottom side of the furnace (to monitor the refractory damage and metal infiltration risks)
g- Thermocouple 15g to measure the temperature of the exit flue gas
h- Thermocouple to measure the flue gas temperature after the heat exchanger
i- Thermocouple to measure the flue gas temperature before the heat exchanger
k- Thermocouple to measure the inlet gas temperature
l- Thermocouple to measure the inlet air temperature
m- Gas/fuel flow rate measurements
n- Air/oxygen flow rate measurements
o- Optionally, sensor indicating furnace tilting and furnace position
p- Sensor indicating the presence of flame
q- Optionally, sensors indicating the furnace weight (on hydraulic pistons)
r- Electromagnetic stirrer power, frequency
s- Optionally, sensor to analyze the chemical composition of the flue gas

The gas furnace control system 2 comprises a furnace control unit comprising inputs connected to the sensors 15 and outputs connected to automated furnace actuation devices such as the stirrer induction coil (if available), door actuation motor (if available), fuel and air control valves to control the gas burner heat output, flue exit vent actuators (if available) and other actionable motors and actuators controlling elements of the furnace.

The furnace control unit further comprises a data output connected to a melt optimization computing system 6. The melt optimization computing system may either be integrated into the furnace control unit, or provided as a computing system separate from the furnace control unit. In the illustrated embodiments, the computing system is illustrated as a separate system from the furnace control unit. In the latter embodiment, the melt optimization computing system 6 may be in the form of a local computing system installed at the site of the furnace, or be in the form of a distributed computing system remote from the site of the furnace and connected to the furnace control unit 4 via a communication network 12, for instance the internet, or a combination of both a local computing system and a remote computing system.

The control system 2 comprises a melt optimization control program installed and executable in the melt optimization computing system 6, and a database 10 including data stored therein from previous melting cycles.

The data of a melting cycle, present or past, may include data from some or all of the sensors 15 and operational data, which may include:
- Type of metal load (scrapes types and morphology) and loading time sequence. These data can possibly be obtained through another program, which calculates the loading composition from available scrapes, or the operator can manually provide these data to the program
- Time of the first loading
- Time to start melting
- Time of transfer (after melting, the liquid metal may be transferred to a holding furnace for further treatment)

The control system 2 further comprises an operator interface 14 for displaying information on the melting process and optionally for allowing the operator to input operational data on the melting process and instructions for operation and control of the furnace. The operational data on the melting process, such as the start or end times, loading of metal into the furnace chamber, operation of the stirrer, or other operations controlled manually by the operator during the melting process may be transmitted to the computing system for analysis by the melt optimization program and/or for storage in the database 10. The instructions for operation and control of the furnace may be inputted into the furnace control unit to control the automated furnace actuation devices.

The operator interface 14, in an embodiment illustrated in figure 6, may include a furnace status panel 16a, a recommendation panel 16b, and a control and further actions panel 16c.

The furnace status panel 16a may comprise various information on the status of the melting process, such as the position of the door (open or closed), the start time, the run time, the temperature of the melt, the estimated fuel or energy consumption, the percentage of melt vs solid (solid fraction), and other status parameters useful for the operator to know.

The recommendation panel 16b may comprise various information on past actions and recommended future actions along a timeline in the melting process for the operator to execute or to control, such as when to actuate the stirrer, when to introduce the thermocouple into the melt, when to clean, when to load additional solid metal into the furnace, and other actions such as the adjustment of the gas burner output.

The control and further actions panel 16c may comprise various information on past actions and future actions, such as the next action to be executed and the timing thereof.

The melt optimization control program comprises a data acquisition module configured to receive data from at least some of the sensors 15, including temperature sensors, a simulation module that is configured to calculate a physical model of heat exchange in the furnace, and a learning algorithm. The calculation of the physical model of heat exchange in the furnace may be used to simulate the melting process to the end of the melt cycle, in particular to estimate parameters such as the solid fraction, melt temperature, and fuel or energy consumption over time. The physical model is adjusted during the melt cycle based on physical measurements of the present state provided by the sensors 15 and optionally by operator inputs, in order to refine the predictions of parameters as the melting cycle progresses based on past information. The learning algorithm processes data from previous melt cycles from the database 10 to determine the efficiency or effectiveness of past actions and based thereon to adjust recommendations for future actions. The prediction and learning algorithms process and output time-based recommendations on actions to be undertaken during the melting process for the operator to execute manually or for automatic execution by the furnace control unit 4.

The data acquisition module captures the measurements of at least some of the sensors 15, especially temperatures, during the melting cycle continuously or intermittently, for instance at predetermined intervals. In parallel to data acquisition, the physical model of heat exchange in the furnace, over a future span of time, is calculated by the simulation module, based on a calculation of heat exchange between the gas burners and the furnace chamber, mutual radiation between the various surfaces, thermal conduction within the various domains, convection within the metal and the air, and oxidation at the top surface of the metal load. The model also takes into account several operations such as: door open or closed, addition of solid or liquid metal, liquid melt stirring, surface oxidation (exothermic) and surface oxide skimming.

The predicted data at the location of sensors from the physical model is compared with measured data from the sensors 15 and allows to adjust some of the parameters such as heat transfer coefficients between the burner and the various surfaces. The adjustments may be made at each data acquisition time or at intervals spanning a plurality of data acquisitions. As the melting cycle progresses, the adjustment becomes more and more accurate as the number of comparison data increases.

Advantageously, the physical model is based on heat exchanges and mass transfer within the furnace and metal load that encapsulates the most important physical phenomena (radiation, conduction, convection). While taking into account the geometry of the furnace, its implementation into a numerical code is made in such an efficient way that the simulation may be calculated with a CPU time that is faster than one step of data acquisition, which may occur typically between every 1 to 10 seconds, and thus also much faster than the whole melting cycle which may typically be a few hours. An example of a one dimensional or two dimensional physical model used by the simulation module according to an embodiment of the invention is described hereafter.

The physical model, on which the invention is based, is sufficiently fast to allow numerical simulation of the whole melting process over a time that is faster than the data acquisition system. Yet, it includes the main physical phenomena involved in the process: combustion of the gas and heat exchange of the fumes, heat exchange between the burner and the various surfaces (furnace walls and vault, metal surface), mutual radiation between them, thermal conduction in the various media below these surfaces, convection in the metallic melt, (exothermic) oxidation at the melt surface, phase transformation and compaction within the metal load during melting. The model accounts for the geometry of the furnace, in particular of the non-parallelepiped pool containing the metal. At the core of the model is the mutual radiation between the various surfaces which is calculated according to the laws of radiation with appropriate viewing factors. Opening of the door, which influences mutual radiation of the furnace and metal surfaces, is accounted for.

The implementation of the model is made according to an implicit time-stepping scheme which removes the stability condition of explicit schemes and allows to have time steps that follow accurately those of the data acquisition system.

Temperature-dependent materials properties controlling radiation (emissivity) and conduction (thermal conductivity) are taken from the literature, while those which are not as well known (e.g. heat transfer coefficients from the burner flames to the various surfaces) can be adjusted on-line during data acquisition with a retro-fit method.

An important advantage of the method of the invention is a unique combination of data acquisition and simplified modelling that is reliable and fast. As the numerical model is sufficiently fast, yet physically based, this allows to make some inverse modelling on line during the melting cycle in order to optimize some of the not so well-known parameters of the process. As this fine tuning of parameters is done during data acquisition, this allows to become increasingly predictive in the future of the melting process. The method thus accumulates during one melting cycle the past experience to predict the future and to minimize in this way the melting cycle, the consumed energy, the amount of CO₂ release. It becomes a guide to the operator for what is happening in the furnace, without opening the front door, and for when making necessary operations such as reloading some more metal and scrapes, skimming the oxide skin, stirring the melted metal, inserting the thermocouple into the melt without breaking it or terminating the melting cycling within the right time and without excess superheat.

The control system according to the invention allows to determine the optimal process sequences and parameters evolving over time to minimize the total cycle time, total energy consumption and dross generation.

An example of a numerical model to simulate a physical model of heat exchanges in a melting furnace according to an embodiment of the invention is described below with reference to figures 1a, 1b, 1c and 3 in particular. The geometry of the furnace being modelled is substantially parallepipedic, however other furnace geometries may be considered and modelled.

In order to optimize melting or remelting furnaces, in particular for the Al industry, a numerical model based on sound physical aspects, has been developed. It is fast and efficient and directly coupled with *in situ* data acquisition, it allows reverse engineering and optimisation to be made on line.

The model takes into account that the furnace comprises a bottom portion containing the metallic melt 1, a moving front door 7 which allows to feed the metal into the furnace in one or several batches, an open space above the metal further delimited by a lateral surface (side wall 5c) and a vault (top wall 5a). Temperature *Tᵥₐᵤₗₜ* is measured in the top wall, and optionally in other positions on the lateral surfaces. Heat is provided by combustion of a gas through one or several gas burners 11. The gas flow *G_{flow}* and gas temperature *T_{gas}* are measured. In many furnaces, fumes resulting from combustion exit though a heat exchanger 17, allowing to preheat fresh air flow *A_{flow}* to an air temperature *Tₐᵢᵣ* which is also measured. The temperature of the metal *Tₘₑₜₐₗ* can be measured with a thermocouple 15d which can be inserted into the melt once it is sufficiently liquid. The model includes three main components:
- A model of combustion
- A model of heat transfers
- A coupling with on-line data acquisition

### Combustion model

This part of the model describes the power input from the reactants and the losses from the combustion products during the operation of the furnace.

Knowing the excess air ratio with respect to the gas *λ* (*λ* = 1 corresponds to no excess) and assuming full combustion of the gas, the stoichiometric reaction of combustion for a gas such as methane may be calculated according to: ${CH}_{4} + 2 λ ⋅ \left({O}_{2}+3.76{N}_{2}\right) = {CO}_{2} + 2 {H}_{2} O + \left(λ-1\right) ⋅ {O}_{2} + 2 λ ⋅ \left(3.76{N}_{2}\right)$

The power exchange *Q*˙ *^{burn}* between the combustion products and the furnace can be readily obtained from the equation: ${\dot{Q}}^{burn} = {\sum }_{p} {\dot{n}}_{p} {h}_{p}^{f} \left({T}_{p}\right) - {\sum }_{r} {\dot{n}}_{r} {h}_{r}^{f} \left({T}_{r}\right)$ where *ṅₚ* and *ṅᵣ* are the molar fluxes of products and reactants, respectively, while ${h}_{p}^{f} \left({T}_{p}\right)$ and ${h}_{r}^{f} \left({T}_{r}\right)$ are the molar enthalpy of formation of each component, taken at their corresponding temperatures, *Tₚ* and *Tᵣ*. In the example of Eq. (1), the reactants are CH₄, O₂, and N₂, while the products are CO₂, H₂O, O₂ and N₂.

The enthalpy of formation of the various chemical species ${h}_{i}^{f} \left({T}_{i}\right)$ (*i* = *r* for reactants and *i* = *p* for products), are calculated from the enthalpy of formation ${h}_{i}^{f} \left({T}_{0}\right)$ at a reference temperature *T*₀*,* according to the equation: ${h}_{i}^{f} \left({T}_{i}\right) = {h}_{i}^{f} \left({T}_{0}\right) + {\int }_{{T}_{0}}^{{T}_{i}} {c}_{pi}^{m} \left(θ\right) dθ$ where ${c}_{pi}^{m}$ is the temperature-dependent specific heat of the considered species *i*, per unit mole. The temperatures *Tᵢ* of the various species in Fig. 1b are: *Tₐᵢᵣ* for air, *T_{gas}* for gas, and *T_{fume}* for the exit fumes.

The molar fluxes of the various species are calculated from the measured flow rates of gas *G_{flow}* and air *A_{flow}*, while their temperatures *Tₐᵢᵣ*, *T_{gas}* are directly estimated from temperature sensors in the respective air and gas conduits. The fraction of fumes going through the heat exchanger 17 is accounted for in the heat balance.

The obtained heat power exchange *Q̇^{burn}* is then used as an input in the numerical simulation of conduction and radiation heat transfers.

### Heat transfer model

### Contribution from the burners

The total heat power exchange *Q̇^{burn}* is attributed to the various furnace surfaces according to adjustable parameters ${α}_{j} \left({{T}_{{j}^{*}}}^{t}, {T}_{flame}\right) .$ In the case of a parallelepipedic furnace, the index "j" can take 6 values corresponding to the metal surface, the vault, the door and the three other lateral surfaces. A surface (j) has a temperature ${{T}_{{j}^{*}}}^{t}$ at a given time *t*, and *T_{flame}* is the temperature of the flame of the burner. The parameters ${α}_{j} \left({{T}_{{j}^{*}}}^{t}, {T}_{flame}\right)$ can be optimized during the process by inverse modelling (or reverse engineering) in order to best fit the measured values (see next section).

Taking into account these coefficients ${α}_{j} \left({{T}_{{j}^{*}}}^{t}, {T}_{flame}\right) ,$ the total flux ${\dot{Q}}_{j}^{burn}$ [W] received by surface *Sⱼ* is given by: ${\dot{Q}}_{j}^{burn} = {α}_{j} {\dot{Q}}^{burn} \frac{{S}_{j}}{{\sum }_{j} {S}_{j}} with \frac{{\sum }_{j} {α}_{j} {S}_{j}}{{\sum }_{j} {S}_{j}} = 1$ or a flux density ${\dot{q}}_{j}^{burn} = {\dot{Q}}_{j}^{burn} / {S}_{j}$ [W/m²] given by: ${\dot{Q}}_{j}^{burn} = {α}_{j} \frac{{\dot{Q}}_{burner}}{{\sum }_{j} {S}_{j}} with \frac{{\sum }_{j} {α}_{j} {S}_{j}}{{\sum }_{j} {S}_{j}} = 1$

### Radiation among the furnace surfaces

At the core of the heat transfer model is a calculation of radiation between the various surfaces (melt, vault, door, lateral walls), radiation being the dominant heat transfer process in a remelting furnace for Al alloys. The model uses a net radiation method, assuming each surface (j) to be grey, with an emissivity ε*ⱼ*(*Tⱼ*), and diffuse. In order to speed up the calculations, the average viewing factors *Fⱼₖ* being surface (j) and surface (k) (see figure 1c) are calculated either by analytical integration for a parallelepipedic furnace or by numerical integration for a more complex furnace shape. It is recalled that the viewing factors *Fⱼₖ* are given by: ${F}_{jk} {S}_{j} = {F}_{kj} {S}_{k} = \frac{1}{π} {\int }_{{S}_{j}}^{ } {\int }_{{S}_{k}}^{ } {dξ}_{j} {dη}_{j} {dξ}_{k} {dη}_{k} \frac{{cos θ}_{j} {cos θ}_{k}}{{r}_{jk}^{2}}$ where (*ξⱼ,ηⱼ*) are two parametric parameters of surface *Sⱼ* (e.g, (*x*,*y*) for *S*₁ in Fig. 2), (*ξₖ*,*ηₖ*) are two parametric parameters of surface *Sₖ* (e.g, (*y*',*z*) for *S*₂ in Fig. 1c), *rⱼₖ*(*ξⱼ,ηⱼ,ξₖ,ηₖ*) is the distance separating the two surface elements, and cos *θⱼ* and cos *θₖ* are the two cosines of the angles between *rⱼₖ* and the outward-pointing normal to each surface (see Fig. 1c). Once these geometrical viewing factors are known, the "radiosity" method allows to calculate the heat exchanged by radiation between the various surfaces. Adding the burner energy input, this allows to obtain the heat flux condition at each surface, at each time step, knowing the surface temperatures ${{T}_{{j}^{*}}}^{t}$ of each surface. One has the boundary condition for a surface (j): ${κ}_{j} \frac{\partial T}{\partial n} {)}_{j} = {ε}_{j} \left({\sum }_{k \neq j}^{{N}_{S}} {F}_{jk} {\dot{q}}_{Tk}^{s} - {σ}_{B} {\left({T}_{j}^{* t}\right)}^{4}\right) + {\dot{q}}_{j}^{burn}$ where *κⱼ* is the thermal conductivity of the material below surface (j), the summation is carried out over the *N_{S}* surfaces of the furnace and melt (6 in the case of a parallelepiped), *σ_{B}* is Stefan-Boltzmann's constant, and ${\dot{q}}_{Tk}^{s}$ is the outcoming radiative flux of facet (k). These fluxes are found by solving the system of equations: ${A}_{jk} {\dot{q}}_{Tk}^{s} = {σ}_{B} {ε}_{j} {\left({T}_{j}^{* t}\right)}^{4}$ where the matrix elements *Aⱼₖ* are given by: $\begin{matrix}{A}_{jk} = 1 & if j = k & ; & {A}_{jk} = - \left(1-{ε}_{j}\right) {F}_{jk} & if j \neq k\end{matrix}$

This situation corresponds to a closed door of the furnace, i.e., the cavity of the furnace corresponds to a closed system for radiation. When the door is open, its radiation is considered separately from the other surfaces of the furnace and the corresponding opening is replaced by a medium of emissivity 1 and a temperature equal to the ambient.

### Heat diffusion from the surfaces

Knowing the heat flow contribution from the burner at each surface (Eq. (5)) and their mutual radiation by solving Eqs. (8), the boundary conditions of Eqs. (7) allow then to solve the heat diffusion in each medium below the *N_{S}* surfaces: $\frac{\partial }{\partial {ζ}_{j}} \left({k}_{j}\frac{\partial {T}_{j} \left({ζ}_{j}, t\right)}{\partial {ζ}_{j}}\right) = \frac{\partial {h}_{j}}{\partial t}$ where *ζⱼ* is the coordinate parameter in the material perpendicular to the surface (j), *Tⱼ*(ζ*ⱼ,t*) is the local temperature at location ζ*ⱼ* at time *t*, and *hⱼ* is the volumetric enthalpy. For the ceramics below the surfaces of the furnace, the volumetric enthalpy is simply given by: ${h}_{j} \left(T\right) = {\int }_{0}^{T} {\left({ρc}_{p}\right)}_{j} \left(θ\right) dθ$ where (*ρcₚ*) is the volumetric specific heat of the material. For the metal itself, the enthalpy accounts also for the latent heat of fusion *L_{f}*: ${h}_{met} \left(T\right) = {{\int }_{0}^{T} \left({ρc}_{p}\right)}_{met} \left(θ\right) dθ + {\left({ρL}_{f}\right)}_{metg ℓ}$ where *g*_{ℓ} is the local volume fraction of liquid metal. Equation (10) (Eq. 10) is solved using an implicit time stepping (also called backward Euler) scheme with the boundary condition at the surface given by Eq. (7) and a boundary condition at the outer surfaces of the furnace given by an imposed temperature.

It may be noted that the diffusion equation may be solved below each surface, taking into account the various thicknesses of different ceramics, with their corresponding properties. For the bottom surface (metal), the diffusion equation within the metal and that for the ceramics below are coupled via a heat transfer coefficient at the metal-ceramic interface.

### Coupling with data acquisition

Since the radiation and diffusion calculations are very fast and efficient, with a time step that can be set equal to that of the data acquisition system, the temperatures *T^{m}*(***r**^{tc},t*) measured at the *N_{tc}* locations ***r**^{tc}* of the thermocouples can be compared with calculated values at the same locations and time *T^{c}*(***r**^{tc}*,*t*). Since these later values are function of some parameters, in particular the coefficients *αⱼ* giving the distribution of the burner power, an inverse algorithm can be used to optimize their choice. More precisely, one tries to minimize the function: $S = {\sum }_{tc = 1}^{{N}_{tc}} {\sum }_{p = 1}^{{N}_{t}} {\left[{T}^{m}\left({r}^{tc}, {t}_{p}\right)-{T}^{c}\left({r}^{tc}, {t}_{p}, \left\{{α}_{j}\right\}\right)\right]}^{2}$ where *Nₜ* is the number of time steps used in the optimisation procedure. This minimum is given by: $\frac{\partial S}{\partial {α}_{k}} = - 2 {\sum }_{tc}^{{N}_{tc}} {\sum }_{p = 1}^{{N}_{t}} \left[{T}^{m}\left({r}^{tc}, {t}_{p}\right)-{T}^{c}\left({r}^{tc},{t}_{p}\left\{{α}_{j}\right\}\right)\right] {X}_{k}^{tc , p}$ where the ${X}_{k}^{tc , p}$ are the sensitivity coefficients of temperature *T^{c}*(***r**^{tc}*, *tₚ*,{*αⱼ*}) with respect to variations of parameters *αₖ*: ${X}_{k}^{tc , p} \frac{\partial {T}^{c} \left({r}^{tc}, {t}_{p}, \left\{{α}_{j}\right\}\right)}{\partial {α}_{k}}$ These coefficients can be calculated numerically by small variations of the parameters *αₖ*.

Turning now to the overall melting process, a melting cycle may comprise the following operations:

### Furnace cleaning

Depending on the operational conditions and the amount of deposited dross on the furnace walls and furnace bottom, a cleaning step may be applied before a melting cycle. This cleaning step is typically required at least twice per week for a furnace in service. In the case that the subsequent melting cycle includes materials with incompatible chemical compositions from materials of the previous melting cycle, a full cleaning procedure may be applied to remove all residual metal from the furnace chamber. Otherwise, it is common that a new melting cycle includes some residuals (for instance about two tonnes of liquid residual metal) from the previous cycle.

### Loading

A typical melting cycle starts with loading. Scrapes and ingot and some master alloys can be loaded directly into the furnace. If the principal metal is aluminium, master alloys may for instance include Cu and Zn. In the case of using scrape with low compacity, the loading cannot usually be carried out in one step. In this case the loading is split into several load packages (for instance between 2 to 6). Each load package will be charged into the furnace during the melting cycle, as soon as free space in the furnace allows for further loading. Load packages may contain liquid aluminium obtained from smelting or recycling process. There are several safety issues regarding the loading procedure. For example it is forbidden to charge big ingot and scrapes into the molten pool (to avoid splashes). The loading of scrapes which are not pre-heated also requires several precautions because humidity may create water vapor explosions.

In order to optimize the melting process, a global objective is to load metal into the furnace as soon as possible, as much as possible, and as quickly as possible. The simulation program according to embodiments of the invention predicts the volume change of scrape during melting and thus predicts the time when there is sufficient space inside the furnace allowing for further loading. This helps to minimize the number of door openings, and thus unnecessary energy loss.

### Stirring

Stirring can be applied during a cycle in order to homogenise the temperature inside the furnace. A stirring is applicable and efficient only if there is enough liquid metal in the furnace.

In order to optimize the melting process, the simulation program according to embodiments of the invention predicts whether or not a stirring is required during a melting cycle and what the optimal time is for stirring based on temperature gradients in the metal load, calculated oxide quantities and calculated coefficients of heat absorption.

### Thermocouple introduction

The liquid metal temperature is one of the most important parameters of the melting process. In order to measure this liquid metal temperature, a thermocouple is introduced into the molten pool. The thermocouple should not be introduced if the amount of remaining solid scrapes is too large due to a risk of breaking the thermocouple. After introducing this thermocouple, the gas burners power can be regulated based on the measured liquid metal temperature.

In order to optimize the melting process, it is desirable to introduce the thermocouple as soon as possible. The simulation program according to embodiments of the invention predicts the optimal time for thermocouple introduction based on the estimation of average metal temperature and liquid fraction over time.

### Skimming

Skimming is applied to remove the oxides that form at the upper surface of the molten pool. The formation of oxides at the upper surface of the pool generates heat but has also an important impact on the heat transfer from burners to metal. Skimming has therefore a significant impact on the furnace efficiency. A normal melting cycle includes at least one skimming step. It is normally performed when the metal is fully molten. In some furnaces, depending on the type of scrapes, skimming might have to be avoided. In the case of formation of significant oxide during the cycle, an early skimming may be applied to remove this oxide layer at the middle of a melting cycle.

In a reverberatory gas/fuel furnace for aluminium melting, it is important to optimize the timing for removal of the dross layer on the metal melt by skimming. The dross layer is made of aluminium oxide which has a high melting point. The dross layer will not melt further, but acts as a heat insulator. If it is allowed to grow too thick, it will insulate the metal melt from the burner flame. The dross will be more heated and more metal will be oxidized. Note that the formation of the oxide skin is exothermic, i.e., generates heat which may be included in the physical model.

In order to optimize the melting process, skimming should thus be applied when a significant amount of oxide has formed and decreases substantially the heat transfer from burners to metal load. In addition, skimming is only possible if there is significant amount of liquid available. The simulation program according to embodiments of the invention predicts the optimal time for skimming based on an estimation of the fraction of liquid metal over time.

### Sampling and alloying

In some metal melting processes, a sample may be taken from the furnace to determine the chemical composition of the melt. Master alloys may be added to the melt to obtain the desired chemical composition.

### End of cycle

The melting cycle ends when the liquid metal has achieved the desirable temperature and chemical composition.

In order to optimize the melting process, increasing the melt temperature above the desired superheat (typically 720°C for aluminium) should be avoided for several reasons: excess of energy consumption, increase of metal oxidation, longer melting cycle, and evaporation of some solute elements (e.g. Zn). Simulation of the melting process with the simulation program according to embodiments of the invention in addition to data acquisition when the thermocouple is inserted into the melt allows to achieve the optimal time-temperature cycle.

A melting process according to an embodiment of the invention is illustrated in figure 7. The melting process may include the following steps:
1- Collecting data from sensors 15 - examples of data measured during a melting cycle are illustrated in figures 4 and 5
2- Calculating inlet power of the burners with fuel, gas, air and oxygen flow rates and their respective inlet temperatures
3- Calculating flue gas chemical composition and flow rates with using data fuel/gas/air /oxygen flow rates with respect to combustion reaction
4- Obtaining flue gas temperature from the sensors
5- Calculating in real-time the gas burners power based on gas/fuel/air/oxygen flow rates, temperatures, using numerical description of combustion
6- Calculating power loss through flue gas using flue gas flow rate and temperature
7- Numerical simulation of the furnace from the beginning of the melting cycle up to the actual time based on the physical model described hereinabove
8- Adjusting the physical model on a real time basis by comparing simulated and measured values such as furnace vault temperature to tune some heat transfer coefficients and some adjustable parameters in the model on a real time basis
9- Determining some process values such as metal temperature, solid, liquid and oxide quantities with the tuned physical model
10- Determining metal load volume and free available space in furnace with the tuned physical model
11- Determining the heat flux (heat transfer coefficients) to the metal load and to the various surfaces of the furnace, with the tuned physical model
12- Calculating heat diffusion in the various walls of the furnace as well as in the metal load (in this case, taking into account mass transfer, e.g. creep of solid aluminium and flow of liquid aluminium)
13- Performing simulations for future times during the melting cycle using the tuned model
14- Predicting the gas / air flow rates evolution for future times with an algorithm with tuned burners power to achieve / maintain either vault or metal desirable temperatures (for example 1100°C for vault before thermocouple introduction and 750°C for metal temperature.)
15- Predicting the evolution of solid, liquid, oxide up to the end of the melting cycle
16- Determining the optimal times for split loading (based on the prediction of free space evolution in the furnace)
17- Determining the optimal time for thermocouple introduction (based on obtaining over 90% liquid fraction or average temperature of 700°C in the metal)
18- Determining the optimal time for stirring (based on temperature gradient in the load and coefficient of absorption)
19- Determining the optimal time for oxide skimming, based on oxide quantities and coefficient absorption and liquid metal quantity
20- Repeating some or all of the above steps at predetermined or regular intervals, for instance every 10 to 60 seconds, in order to update values

Figure 5 shows a time-sequence of temperatures actually measured in a furnace by the data-acquisition system and simulated with the physical model. It shows the temperatures of the furnace vault and of the metal bath. Please note that the temperature of the bath is measured only when the thermocouple is plunged into the melt. The events associated with the opening of the furnace door are clearly visible. During the door opening, the thermocouple is removed from the melt, thus explaining the fast temperature decrease, in order to enable mechanical stirring._

### List of references:

**Metal 1**
   Melt
      Melt surface 1a
   Solid
      Ingots
      scrape
**Furnace 3**
   Walls 5
      Top wall 5a
      Bottom wall 5b
      Side walls 5c
   Door 7
      Sliding door
   Furnace chamber 9
   Gas burners 11
   Flue gas exit 13
      Heat Exchanger 17
   Stirrer 17
**Control System 2**
   **Sensors 15**
      Temperature sensors
         Thermocouple 15d to measure the metal temperature
         Thermocouple 15e to measure the temperature on a top side of the chamber
         Thermocouple 15f to measure the temperature on the bottom side of the furnace
      Door sensor
         Sensor 15a indicating that the furnace door is fully open
         Sensor 15b indicating that the furnace door is fully closed
      Sensor to measure the inner furnace pressure
      Flue gas sensor
         Thermocouple 15g to measure the temperature of the exit flue gas
         Thermocouple to measure the flue gas temperature after the heat
      exchanger
         Thermocouple to measure the flue gas temperature before the heat
      exchanger
      Gas sensor
   **Furnace control unit 4**
      Inputs
      Outputs
   **Melt optimization computing system 6**
      Inputs
      Outputs
      Server 8
      communications network 12
      Database 10
      Melt optimization control program
         Simulation module 18a
         Learning module 18b
      Operator interface 14
      Furnace status panel 16a
         Recommendation panel 16b
         Control and further actions panel 16c

## Claims

1. A method of controlling a metal melting process in a gas furnace (3) with a control system (2), the gas furnace comprising a furnace chamber (9) enclosed by walls (5a, 5b, 5c) and a door (7), gas burners (11) configured to heat the metal (1) loaded in the chamber, a flue gas exit (13) and a plurality of sensors (15) including at least one temperature sensor at a top wall (5a) of the furnace chamber and at least one temperature sensor (15d) to measure the metal temperature in its melted state, the method comprising:
a) receiving in the control system during the melting process, process parameter measurements from said sensors including at least one temperature sensor,
b) simulating in the control system a numerical physical heat exchange model in the furnace including radiation between walls and the metal, conduction though the metal and walls, and convection in the furnace chamber including calculating a temperature at a position in the furnace corresponding to said at least one temperature sensor,
c) comparing the data obtained from the simulated physical heat exchange model with data obtained from the sensor measurements,
d) tuning at least one adjustable parameter of the physical heat exchange model to reduce the difference between compared data,
e) based on the tuned simulated physical heat exchange model, calculating in the control system the change over time of the process parameters, including at least one process parameter which is not directly measured up to the end of the cycle,
f) transmitting to an operator interface (14) of the control system, information on the change over time of predicted process parameters and at least one recommendation for executing a future operation in relation to the furnace at a recommended time.

2. The method according to any preceding claim, wherein the process parameters measured and received by the control system and included in the numerical model further include :
- a flue gas exit temperature (*T_{fume}*),

3. The method according to any preceding claim, wherein the process parameters measured and received by the control system and included in the numerical model further include :
- a burner gas inlet temperature (*T_{gas}*)
- a gas flow rate (*G_{flow}*).

4. The method according to any preceding claim, wherein the process parameters measured and received by the control system and included in the numerical model further include :
- an air inlet temperature (*Tₐᵢᵣ*)
- an air flow rate (*A_{flow}*).

5. The method according to any preceding claim, wherein the process parameters measured and received by the control system and included in the numerical model further include any one or more of:
- a chemical composition of at least one component (such as CO₂) of the flue gas,
- a gas pressure inside the furnace chamber,
- a furnace bottom wall temperature.

6. The method according to any preceding claim, wherein the simulated physical heat exchange model includes calculating in the control system the heat exchange when the door is opened and including the opening of the door in the evolution of the process parameters.

7. The method according to any preceding claim, wherein the recommended future operation includes any one or more of the operations of:
- loading solid metal in the furnace,
- skimming dross on the surface of the molten metal,
- stirring the molten metal in the furnace,
- introducing a thermocouple (15d) in molten metal,
- changing the heat output of the gas burners (11),
- introducing chemicals in the furnace,
- introducing alloys in the furnace,
- stopping the melting process.

8. The method according to any preceding claim, wherein the information on the change over time of predicted process parameters transmitting to the operator interface (14) includes a plurality of recommendations for executing said future operations at recommended times up to an end of the melting process.

9. The method according to any preceding claim, wherein generating the recommended future operation and recommend timing thereof includes accessing a database (10) storing past melting process parameters and executing a learning algorithm on said past melting process parameters.

10. The method according to any preceding claim, wherein operator feedback on operations on the furnace are input into the operator interface and transmitted from the operator interface to a server of the control system.

11. The method according to the preceding claim, wherein operator feedback includes information on whether or not operational procedures were executed at the recommended times or postponed.

12. Control system (2) for a gas furnace for melting metal, adapted to carry out the process according to any one of the previous claims, comprising a melt optimization computing system (6) including:
- a melt optimization control program stored in a memory of the computing system and executable by a processor of the computing system, the melt optimization control program comprising an acquisition module configured to receive process parameters from the sensors, including at least one top wall temperature measurement and at least one molten metal temperature measurement, and a simulation module (18a) configured to calculate a physical heat exchange model in the furnace including radiation between walls and the metal, conduction though the metal and walls, and convection in the furnace chamber including calculating a temperature at a position in the furnace corresponding to said at least one temperature sensor, the melt optimization program configured to compare acquired process parameters with process parameters calculated by the numerical physical heat exchange model and to tune the model by adjusting at least one parameter thereof in order to reduce the difference between measured and calculated process parameter values; and
- an operator interface (14) comprising a display, configured to receive and display information outputted by the melt optimization program, including information on the change over time of predicted process parameters and at least one recommendation for executing a future operation in relation to the furnace at a recommended time.

13. Control system according to the preceding claim, wherein the operator interface is arranged to display a furnace status panel (16a) providing information on the status of process parameters and a recommendation panel (16b) providing information on the recommended future operations and the timing thereof.

14. Control system according to the preceding claim wherein the operator interface is arranged to display a control and further actions panel (16c) providing information on the next recommended operation and the timing thereof.

15. Control system according to any preceding claim, further comprising a database (10) in which process parameters of past melting processes are stored, and a learning module (18b) receiving data from the database (10).
